

## UNITED STATES PATENT OFFICE.

WALTER JAMES STEVENSON, OF LONDON, ENGLAND.

## MANUFACTURE OF ARTIFICIAL SILK FROM ACETYL CELLULOSE.

No Drawing.

Application filed March 13, 1923. Serial No. 624,822.

*To all whom it may concern:*

Be it known that I, WALTER JAMES STEVENSON, a subject of the King of Great Britain and Ireland, and a resident of

London, England, have invented a certain new and useful Improvement in the Manufacture of Artificial Silk from Acetyl Cellulose, of which the following is a specification.

For the purposes of this invention I take acetyl cellulose made preferably under my British Patent No. 130,029 of 1919, which I dissolve in acetone or other suitable solvents from which is removed every trace of suspended or insoluble matter, and putting this in containers from which it is forced under pressure by compressed air, or pump, through fine orifices. The orifices are submerged in a decomposing solution of sodium sulphate which removes the solvent, and leaves a continuous thread of fibre. This fibre is passed round a bobbin, or deposited into some form of yarn container having a

circular motion. The number of filaments are dependent upon the thickness of the yarn which it is intended to produce. The fibres are then dried and wound on to bobbins. The artificial silk thus made is not regenerated cellulose but cellulose containing acetic acid.

I am aware that it has been already proposed to make artificial silk by squirting solutions of cellulose acetate into salt solutions but I make no broad claim thereto.

I claim:

The manufacture of artificial silk from acetyl cellulose by dissolving same in acetone or other suitable solvents, and after filtration forcing same through fine orifices or openings, into a decomposing bath containing sodium sulphate, which forms a continuous thread or fibre.

In testimony whereof I have affixed my signature hereto this 26th day of February, 1923.

WALTER JAMES STEVENSON.